

# United States Patent [19]

Schebece et al.

[11] Patent Number: 4,554,097

[45] Date of Patent: \* Nov. 19, 1985

[54] ELASTIC DETERGENT PRODUCT  
CONTAINING ANIONIC AND  
AMPHOTERIC SYNTHETIC ORGANIC  
DETERGENTS

[75] Inventors: Frank Schebece, Edison; John C. Carson, Jr., Manasquan Park, both of N.J.

[73] Assignee: Colgate-Palmolive Company, New York, N.Y.

[\*] Notice: The portion of the term of this patent subsequent to Jan. 1, 1997 has been disclaimed.

[21] Appl. No.: 594,971

[22] Filed: Apr. 19, 1984

## Related U.S. Application Data

[63] Continuation of Ser. No. 326,582, Dec. 2, 1981, abandoned, which is a continuation of Ser. No. 746,995, Dec. 2, 1976, abandoned.

[51] Int. Cl.<sup>4</sup> ..... C11D 1/50; C11D 17/00

[52] U.S. Cl. ..... 252/542; 252/DIG. 16; 252/117; 252/121; 252/122; 252/132; 252/134; 252/89.1; 252/546; 252/551; 252/535

[58] Field of Search ..... 252/89, DIG. 16, 174, 252/134, 132, 121, 122, 542, 546, 550, 551, 108, 117, 535

## References Cited

### U.S. PATENT DOCUMENTS

3,442,812 5/1969 Barnhurst ..... 252/DIG. 16  
3,689,437 9/1972 McLaughlin ..... 252/335  
3,708,425 1/1973 Compa et al. ..... 252/DIG. 16

## FOREIGN PATENT DOCUMENTS

731396 6/1955 United Kingdom ..... 252/DIG. 16  
1194861 6/1970 United Kingdom ..... 252/DIG. 16

Primary Examiner—Edith Buffalow  
Attorney, Agent, or Firm—Herbert S. Sylvester; Murray M. Grill; Norman Blumenkopf

## [57] ABSTRACT

An elastic detergent product which may also be used by children as a toy or plaything while taking a bath, includes a mixture of anionic and amphoteric synthetic organic detergents, gelatin and water. The products are substantially form-retaining and although they wear away during use, substantially retain their initial forms and elasticities for major proportions of their useful lives. They are easily manufactured and during the manufacturing process are moldable to finely figured and detailed shapes. Because of their elasticity they are resistant to breakage during shipping and use and because of their contents of both synthetic anionic and amphoteric organic detergents they exhibit less surface tackiness than other elastic detergent products or bars in which similar proportions of gelatin and water are present. In an improved process for the manufacture of such products having a lesser tendency to shrink upon prolonged exposure to the atmosphere, during the blending of the various product components heating is employed and is continued for a long enough time to evaporate a substantial proportion of water from the mixture, after which the composition may be poured into molds and solidified.

15 Claims, No Drawings

**ELASTIC DETERGENT PRODUCT CONTAINING  
ANIONIC AND AMPHOTERIC SYNTHETIC  
ORGANIC DETERGENTS**

This is a continuation of application Ser. No. 326,582, filed Dec. 2, 1981 now abandoned which is a continuation of Ser. No. 746,995 now abandoned.

This invention relates to elastic detergent products. More particularly, it relates to detergent products or bars intended for conventional toilet soap uses, either as hand "soaps" or bath or shower "soaps", which are elastic in nature and which include both synthetic organic anionic and amphoteric detergents. Such elastic detergent bars are less tacky than various other gelatin-based bars containing only either anionic or amphoteric detergent and such improved surface characteristic, together with their "squeezability", which makes them like a plaything for children, help make bathing more pleasant both for the child and his parent. Additionally, they foam better than other detergent bars.

Soap, synthetic organic detergent and soap-synthetic detergent bars and cakes have been made from literally thousands of different materials. It has long been known to incorporate perfumes, colorants, abrasives, bleaches, fillers, emollients and bodying agents in soap bars and gelatin is one of the bodying or binding agents that has been employed. Soap bars have usually contained glycerol and water, both of which are produced and utilized in various soapmaking processes when soaps are produced by the saponification of triglycerides. U.S. Pat. No. 2,360,920 discloses the production of soap buds from an aerated aqueous solution of soap containing glycerine and a demulcent, such as may be made from a mixture of Irish moss and gelatin. U.S. Pat. No. 3,698,437 teaches the manufacture of malleable and non-hardenable detergent products from certain percentages of a fatty acid isethionate, water, gelatin, hydrocarbon and filler. The resulting bars, which may also contain glycerol or propylene glycol and other adjuvants, are said to be moldable and extrudable but not elastic. British Pat. No. 731,396 describes a shaped soapless organic detergent composition in which the soapless detergent, such as triethanolamine alkylbenzene sulfonate, is dispersed in a gelatin gel. Aeration of the gel to produce a frothy product is suggested, as are the additions of various builders, fillers, nonionic detergents, etc. In copending U.S. Pat. No. 4,181,632, issued Jan. 1, 1980, which was filed on Dec. 2, 1976, the same day as the effective date of the present application, by Frank Schebece, improved synthetic organic detergent bars based on synthetic anionic detergent and cross-linked or denatured gelatin are described, as are detergent bars based on amphoteric detergents, with or without such cross-linking and/or denaturing agent(s). However, that application does not describe mixtures of synthetic organic anionic and amphoteric detergents in aqueous gelatin-based products and the unexpectedly beneficial advantages thereof.

Although the prior art has recognized that gelatin may be included in detergent compositions which may be desirably molded or shaped to bar or cake form and although the Schebece application mentioned teaches the employment of amphoteric detergents as the synthetic organic detergent component of such a bar the art did not describe nor suggest the bars of this invention wherein both anionic and amphoteric synthetic organic detergents are utilized. Furthermore, it did not suggest

the advantages obtained due to such composition nor by the invented process wherein the moisture content of a composition of this invention is intentionally diminished to improve the ultimate properties of the molded bar.

5 In accordance with the present invention an elastic detergent product comprises about 10 to 80% of a mixture of anionic and amphoteric synthetic organic detergents in a proportion between about 1:5 and 5:1, about 10 5 to 30% of gelatin and about 5 to 60% of water. In preferred formulations the anionic detergent is a monoglyceride sulfate or a triethanolammonium higher fatty 15 alcohol sulfate and the amphoteric detergent is an imidazolinium betaine or a betainiminodipropionate, although betaminopropionates may also be employed. In 15 the process embodiment of the invention such a product is made with a moisture content of about 5 to 40% by heating a mix containing more water so as to evaporate off from it about 15 to 50% of the weight of the mixture, as water, after which the composition may be deaerated (an optional step, but preferred), poured into a mold, solidified and removed from the mold, ready for use.

The anionic synthetic organic detergents of this invention include sulfated, sulfonated and phosphonated hydrophobic moieties, especially those which include higher hydrocarbyl groups (preferably fatty), such as alkyl groups of 8 to 20 carbon atoms, preferably of 10 to 18 carbon atoms. These compounds are usually employed as their water soluble salts, such as salts of alkali metals, e.g., sodium, potassium and triethanolamine and ammonia. For the present compositions these salts will usually be either sodium, potassium or triethanolamine salts and of these the triethanolamine (or triethanolammonium) salts will often be preferred. Among the various types of synthetic anionic organic detergents which 25 may be useful are the linear higher alkylbenzene sulfonates, especially those of 12 to 15 carbon atoms, e.g., sodium linear tridecylbenzene sulfonate; paraffin sulfonates; olefin sulfonates, higher fatty alcohol sulfates; monoglyceride sulfates, especially the sulfated monoglycerides of coconut oil, tallow, hydrogenated coconut oil, hydrogenated tallow and synthetic higher fatty acids of 8 to 20 carbon atoms, e.g., sodium coconut oil monoglyceride sulfate, ammonium cocomonoglyceride sulfate; corresponding sulfates and phosphonates and other equivalent organic sulfonates, in most of which the lipophilic group includes a chain of 10 to 18 carbon atoms. In the above description and elsewhere in the specification and in the claims when a material is characterized as a "monoglyceride sulfate" such terminology is intended to describe higher fatty acid monoglyceride sulfates wherein the higher fatty acid is of 8 to 20 carbon atoms, preferably of 10 or 12 to 18 carbon atoms, such as lauric acid, myristic acid, palmitic acid, stearic acid and oleic acid. Additionally useful are the sulfates and sulfonates of nonionic detergents and of nonionic surface active agents, in which products the nonionic base will normally be a polyethylene oxide condensation product of a higher fatty alcohol, such as a condensation product based on a higher fatty alcohol of 10 to 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 969

While sodium lauryl sulfate is an anionic synthetic organic detergent which may be employed, preferably in minor proportion with other anionic synthetic organic detergents in the present compositions, its use is usually not preferable and the corresponding triethanolammonium salt is normally used instead because it can produce a clear bar of good washing and foaming ability which is also stable on storage and maintains its elasticity during use.

The amphoteric detergents which may be utilized to manufacture the elastic detergent bars of this invention include such compounds as Deriphat ® 151, which is sodium N-coco-betaaminopropionate (manufactured by General Mills, Inc.), Deriphat 160, a partial sodium salt of N-lauryl-betaiminodipropionate, and other 15 betaaminopropionates and betaiminodipropionates, Miranol ® C2M (anhydrous acid form, 1-carboxymethyl-1-carboxyethoxyethyl-2-coco-imidazolinium betaine), the water soluble salts thereof, especially the triethanolammonium salt, and other imidazolinium betaines, and other of the various known amphoteric, described in McCutcheon's *Detergents and Emulsifiers*, 1973 Annual and in *Surface Active Agents*, Vol. II, by Schwartz, Perry and Berch (Interscience Publishers, 1958), the descriptions of which are incorporated herein 20 by reference. For example, Deriphats 151C, 154, 160, 160-C and 170-C, and Miranols C2M, S2M and SHD Conc. may be employed. Additionally, even liquid amphoteric detergents may be used, at least in part, e.g., up to 25 or 50% of the amphoteric detergent content. The 25 recited incorporated references also contain extensive descriptions of various suitable anionic detergents and of nonionic and cationic detergents which may be employed in small proportion(s) in the present compositions. The various long chain substituents in the mentioned amphoteric are of 8 to 20 carbon atoms, preferably of 10 to 18 carbon atoms and most preferably are lauryl and coco.

The nonionic detergents, while not required components of the invented products, may be present in relatively small proportions therein in replacement of some of the anionic or amphoteric detergents. The nonionics are preferably solid or semi-solid at room temperature, more preferably solid, and include but are not limited to ethoxylated aliphatic alcohols having straight or 40 branched chains (preferably straight chain) of from about 8 to 20 carbon atoms, with about 3 to about 30 ethylene oxide units per molecule. Particularly, suitable nonionic detergents of such type are manufactured by Shell Chemical Company and are marketed under the 45 trademark Neodol ®. Of the various Neodols available, Neodol 25-7 (12-15 carbon atoms chain higher fatty alcohol condensed with an average of 7 ethylene oxide units per mol) and Neodol 45-11 (14-15 carbon atoms chain higher fatty alcohol condensed with an average of 55 11 ethylene oxide units per mol) are particularly preferred. Another suitable class of ethoxylated aliphatic alcohol detergents is made by Continental Oil Company and is sold under the trademark Alfonic ®. Of the Alfonics the most preferred is Alfonic 1618-65, which is a mixture of 16 to 18 carbon atoms primary alcohols ethoxylated so as to contain 65 mol percent of ethylene oxide. Additional examples of nonionic synthetic organic detergents include those marketed by BASF Wyandotte under the trademark Pluronic ®. Such compounds are made by condensation of ethylene oxide with a hydrophobic base formed by condensing propylene oxide with propylene glycol. The hydrophobic

portion of the molecule has a molecular weight of from about 1,500 to 1,800 and the addition of polyoxyethylene (or ethylene oxide) to such portion increases the water solubility of the molecule as a whole, with the detergent being a solid at room temperature when the polyoxyethylene content is above 50% of the total weight of the condensation product. Such a nonionic detergent is Pluronic F-128 but F-68 may also be employed. Also useful nonionic detergents are the polyethylene oxide condensates of alkyl phenols, such as the condensation products of such compounds wherein the alkyl group contains about 6 to 12 carbon atoms, in either a straight chain or branched chain configuration, with 5 to 25 mols of ethylene oxide per mol of alkyl phenol. The alkyl substituents in such compounds may be derived from polymerized propylene or may be diisobutylene, octene or nonene, for example.

Representative cationic detergents, which usually also possess antibacterial (and fabric softening) properties, include di-higher alkyl di-lower alkyl ammonium halides such as distearyl dimethyl ammonium chloride, and 2-heptadecyl-1-methyl-1-[2-stearoylamido)ethyl]-imidazolinium methyl sulfate. The higher alkyls thereof are of 8 to 20 carbon atoms, preferably 12 to 18 and the lower alkyls are of 1 to 4 carbon atoms, preferably 1 and 2. Such materials are normally omitted from anionic detergent based products but may be employed in small proportions in mixed anionic-amphoteric detergent bars, especially when they contain more amphoteric detergent than anionic detergent and when the proportion of anionic detergent is relatively small.

Gelatin, a complex mixture of collagen degradation products of molecular weight in the range of about 30,000 to 80,000 and higher, depending on the hydrolytic conditions to which it has been subjected, is a vital constituent of the present compositions. Apparently because of its outstanding ability to form reversible gels, its high viscosity and the excellent strengths of films thereof, it helps to make a detergent bar which is of satisfactory strength and cleaning power, due to gradual dissolution of the ordinarily extremely soluble synthetic organic detergent component, and yet, which does not produce objectionable and unacceptable soft gels at bar surfaces which have been moistened. Additionally, and a major advantage of the present invention, the combination of gelatin and synthetic organic detergents, in the presence of water and preferably also in the presence of a lower dihydric or polyhydric alcohol or other suitable plasticizer, and often too, a cross-linking agent or denaturant, yields elastic products. The elastic detergent bars made are sufficiently elastic so that a bar 2 cm. thick can be pressed between thumb and forefinger to a 1 cm. thickness and will immediately (within five seconds) return to the 2 cm. thickness or at least to within 1 mm. thereof, upon release of pressure.

The gelatin employed is essentially colorless and free from odor. It is amphoteric (about 45 milliequivalents of amino functions and about 70 milliequivalents of carboxyl functions per hundred grams thereof). It is normally used in formulating as a dry granular product which is crystalline in appearance although it is really amorphous. It is insoluble in cold water but swells rapidly in the presence of water until it has imbibed about 6 to 8 times its weight thereof and it melts to a viscous solution in water when warmed to above 40° to 45° C. Gelatins are classified as either type A or type B, the former being from acid-cured stock, with an isoelectric point of about 8.3-8.5 and the latter being of alkali-

cured stock, with an isoelectric point of about 4.8-5.0. Type A gelatins are preferred for the present applications but type B gelatins may also be used, as may be mixtures of the two. The gelling powers of gelatins are normally measured by the Bloom test. Often too, viscosity will also be employed to characterize a gelatin and a gel strength:viscosity ratio may be specified, e.g., 3:1 to 5:1. Gel strengths will range from 100 to 300 g. Bloom but will usually be in the range of 150 or 200 to 300, with gelatins of Bloom values of 225 g. and 300 g. being employed in the examples herein. The type A gelatins will generally be utilized with the usual detergent bar constituents normally intended for employment in neutral or slightly basic aqueous media, and the type B gelatins will be preferred when acidic conditions are expected to be encountered.

Cross-linking agents for gelatin and for other proteins are metal salts which cross-link various gelatin molecules, apparently by reacting with free carboxyl functions thereof. This class of compounds is well known and the salts employed are usually those of aluminum, calcium, magnesium and/or zinc that are soluble in aqueous media. In such salts the preferred anions are chloride, bromide, iodide, sulfate, bisulfate and acetate but other suitable anions may also be included. Examples of such salts include potassium aluminum sulfate hydrate [alum,  $KAl(SO_4)_2 \cdot 12H_2O$ ], aluminum chloride, other alums, calcium chloride, magnesium sulfate and zinc acetate. Also useful for cross-linking is formaldehyde, usually as formalin. 0.1 To 1% of formaldehyde is normally adequate. Although the presence of a cross-linking agent is often highly desirable in the formulations of the invented bar compositions, especially those based on anionic detergents primarily, it has been found that such are not as important or useful in those compositions based primarily on amphoteric detergents.

Instead of or in addition to a cross-linking agent there may be employed with the gelatin of the present compositions a denaturant. Such a compound also helps to reduce solubility of gelatin at and near its isoelectric point and inhibits crystallization. Although denaturation may be effected by various materials, including various detergents, ethanol, acetone, strong acids and strong alkalies, chemical denaturation, usually by urea, dextrose or guanidine hydrochloride is preferred and of these compounds urea is by far the preferred. Both cross-linking and denaturation and the combination thereof are helpful in producing a lastingly elastic detergent bar of desired properties, suitable for repeated and satisfactory cleaning applications, but neither cross-linking agents nor denaturants for gelatin are required to make a satisfactory elastic detergent bar of the present invention.

The lower dihydric and/or polyhydric alcohol component(s) of the present bars functions as a mutual solvent and plasticizer for the bar components, especially the gelatin. It facilitates solubilization of the detergent at a desired rate and maintains the surface of the bar soft. If the bar became objectionably hard at portions thereof this could be cause for rejection of it by consumers. Such alcohol also helps to distribute the various components evenly throughout the bar or cake. Although a variety of lower dihydric or polyhydric alcohols may be employed, including various sugars and sugar alcohols, having up to 6 carbon atoms and up to 6 hydroxyls per molecule, the most preferred are those of 2 to 3 carbon atoms and 2 to 3 hydroxyl groups per molecule. Such compounds include propylene glycol

(1,2-dihydroxypropane or 1,2-propylene glycol), trimethylene glycol (1,3-propylene glycol) and glycerol, of which 1,2-propylene glycol, glycerol and mixtures thereof are preferred. Other useful solvents are the Cellosolves®, the mono- and di-lower alkyl ethers of ethylene glycol. Additionally, sometimes monohydric alcohols, such as ethanol, are useful, primarily as supplementary solvents.

The water employed is preferably deionized water which will normally contain less than 10 parts and preferably less than 1 part per million of hardness, as calcium carbonate, but normal city waters may also be utilized, such as those having hardnesses in the range of 10, 20 or 50 to 150 or 300 p.p.m., as  $CaCO_3$ .

With the basic elastic detergent bar composition there may be present various adjuvant materials in minor proportions to contribute their particular properties to the final product. Among such adjuvant materials are functional and aesthetic adjuvants, such as: perfumes; pigments; dyes; optical brighteners; skin protecting and conditioning agents, e.g., lanolin, solubilized lanolins; bactericides; chemical stabilizers, e.g., sodium bisulfite; foam stabilizers, e.g., lauric myristic diethanolamide; buffering agents and pH adjusters, e.g., triethanolamine, hydrochloric acid, phosphates; bodying agents, e.g., clays; superfatting agents, e.g., stearic acid; anti-redeposition agents and soil dispersants, e.g., polyvinyl alcohol, sodium carboxymethyl cellulose; gums, e.g., sodium alginate, which also functions as a slip improving agent; and abrasive or scouring components, e.g., silex. Usually the present bars do not and should not contain any fillers or builder salts other than those which may accompany, usually unavoidably, other components of the product. However, in certain circumstances, as when bars for heavy duty laundry use are made, it may be desirable to add fillers, such as sodium sulfate and sodium chloride and builder salts, such as pentasodium tripolyphosphate, sodium carbonate and sodium silicate.

The proportions of the various components of the present elastic detergent bars should be kept within ranges to be given to obtain the best results and to produce a bar which will be desirably elastic, useful in place of conventional soap, soap-detergent and detergent bars and which will possess improved properties, such as a lesser tendency to slough when in contact with water, compared to such more conventional bars. The synthetic organic detergent component, the mixture of anionic and amphoteric detergents, will be about 10 to 80% of the product, preferably 35 to 65 or 70% and more preferably 35 to 55% thereof. The content of cross-linking agent and/or denaturing agent for the gelatin, when present, is usually 0.1 to 5%, preferably 1 to 3% and more preferably 1 to 2% total. Normally the percentage of cross-linking agent will be 0.1 to 5%, preferably 1 to 2% and that of the denaturant will be 0.5 to 2%. The gelatin, preferably type A gelatin of 225 to 300 g. Bloom, will be about 5 to 30%, preferably 7 to 25% and more preferably about 10 to 20% of the finished bar or cake and the moisture content will be about 5 to 60%, preferably 10 to 40% and more preferably 10 to 30%, e.g., 25%.

The lower dihydric or polyhydric alcohol, which may be omitted if syneresis problems are encountered (usually due to a high percentage of normally liquid components of the product), will normally be present in the range of 3 to 20%, preferably 10 to 18%, e.g., 15%.

The total proportion of various adjuvants present, including any builders and fillers, will normally not exceed 10%, preferably will be less than 5% and more preferably will be less than 2%, with the proportion of any particular adjuvant usually being held to less than 5%, preferably less than 2% and more preferably less than 1%.

The manufacture of the present elastic detergent bars is comparatively simple, requiring only the mixing together of the components under such conditions that the gelatin will form a gel with water and/or with any other components present. For example, all the components of a particular detergent composition may be mixed together and heated, with stirring, to dissolve the gelatin. Alternatively the gelatin may be first dissolved in water and the other components may then be admixed or other operative mixing sequences may be adopted. If the components are soluble the product may be transparent or at least translucent but if insoluble ingredients are employed, which may be done intentionally, an opaque gel results. To clarify transparent gels and to increase the strengths and densities thereof these may be deaerated or degassed under vacuum or by allowing the hot or warm liquid to stand until it becomes clarified. The solution or dispersion may then be poured into suitable molds, chilled and thereby solidified. Although gelatin dissolves at temperatures above 40° or 45° C. it is normally undesirable to heat it to a temperature above 100° C. and preferably dissolving will take place at a temperature in the range of about 50° to 90° or 95° C., more preferably about 60° to 80° C., over 3 to 30 minutes. Molds will be at a temperature of 5° to 20° C., preferably 5° to 15° C. After the gelatin has completely set, which may take from about one minute to an hour, usually taking from three to ten minutes, the elastic detergent bar or cake may be removed from the mold and packed or it may be allowed to be warmed to room temperature before packing, at which temperature it still remains firm, yet elastic.

In a preferred process embodiment of the invention a firmer bar is made which has lesser tendency to shrink on storage and develop syneresis. Such a bar may contain: 10 to 80% of the mixture of anionic and amphoteric synthetic organic detergents in a proportion between about 1:5 and 5:1, preferably 35 to 65% of such mixture in a proportion within the range of 1:4 to 2:1, and more preferably the anionic detergent is triethanolammonium lauryl sulfate and the amphoteric detergent is triethanolammonium 1-carboxymethyl-1-carboxyethoxyethyl-2-coco-imidazolinium betaine; 5 to 30% of gelatin, preferably 7 to 25% thereof and more preferably the gelatin is a type A gelatin of 150 to 300 g. Bloom; and 5 to 40%, preferably 10 to 40% and more preferably about 10 to 25 or 30% water. In the improved process the components mentioned and any other solvents, plasticizers, cross-linking agents, denaturants and adjuvants may be mixed together and the gelatin is dissolved in the mixture or in the water thereof, with heating. Preferably the total proportion of water plus solvent plus plasticizer present will be in the ranges previously mentioned for water alone in the final bar but during dissolving of the gelatin, during which the temperature may be raised, as previously described, enough additional water will be employed initially to facilitate solution of the gelatin and it will be heated for a period sufficient to drive off water (or water plus solvent, etc.) to the extent of 15 to 50% of the weight of the mixture, preferably 20 to 40% thereof. In addition

5 to heat, vacuum may be used to facilitate removal of the moisture and any volatile solvent present, such as ethanol. Normally the additional heating to remove moisture, depending on whether or not vacuum is also employed, may take from one minute to thirty minutes and preferably will take from one minute to fifteen minutes. After removal of the moisture the mix may be molded in the manner previously described, but yields the superior product mentioned.

8 The elastic detergent bars of this invention possess an obvious novelty advantage over ordinary soap or detergent bars. They are especially attractive to children when molded into various special shapes, such as the shapes of storybook or cartoon characters, animals, etc., and promote the enjoyment of bathing by infants and young children. The elastic nature of the product allows a controlled dispensing of detergent and other foaming materials onto the skin or into the bath water in response to repeated squeezings and relaxings of the bar. Thus, the utilitarian detergent is also a delightful toy. However, the product has various other advantages apart from its play value. Thus, the presence of the gelatin adds a skin care ingredient to the composition and because of the bar's elasticity breakage during shipment and on storage are minimized. Furthermore, large quantities of synthetic organic detergent may be present in the composition without the need for extensive use of waxes, plasticizers, bodying agents, etc., to control the dissolving thereof and give them desirable tactile properties and good appearances. The bars do not slough excessively, as often do detergent and soap bars and additionally, they maintain substantially their original shapes during use, continually dispensing detergent in response to compression and expansion and rubbing against areas to be cleansed. They have a different "feel" than soap when contacting the skin and this better contact assists in cleaning. The detergents in the bars or other shaped articles are readily released at temperatures of 25° to 40° C. and higher and for cold water washing, at temperatures of 10° C. and less, more soluble and lower Bloom value gelatins can be employed, with appropriate solvents and adjuvants, to help release the detergent. When made by the preferred process, wherein the percentage of moisture in the final product is limited to 40%, and preferably is about 25%, any tendency of the bar to shrink on storage is diminished and a firmer product results. Additionally, surface tackiness is noticeably decreased and the bar foams better than corresponding anionic and amphoteric bars, respectively.

It is to be understood that within the proportions of components given variations may be made to best promote desired properties of the bars manufactured and similarly, processing modifications may also be effected. Thus, proportions of gelatin, detergent, water, cross-linking agent, denaturant, plasticizer and adjuvants may be adjusted, as may be the types of such materials. For example, if the bar is too soft an increase in the solids content and especially in the gelatin content may be desirable and the gelatin type may be changed to that of a higher Bloom value to increase the firmness of the product. Also, in such a case it may be desirable to utilize more cross-linking agent and/or denaturant. If the bar is too firm, reverse adjustments may be made. Those of skill in the art, with this specification before them, will be able to modify the properties of the described compositions to make them conform to

desirable product standards and similarly will be able to modify the processes described.

The following examples illustrate but do not limit the invention. Unless otherwise indicated all temperatures are in °C. and all parts are by weight.

#### EXAMPLE 1

|                                                                                                                                        | Percent |
|----------------------------------------------------------------------------------------------------------------------------------------|---------|
| Triethanolammonium lauryl sulfate                                                                                                      | 8.0     |
| Gelatin (300 g. Bloom type A)                                                                                                          | 10.0    |
| Propylene glycol                                                                                                                       | 10.0    |
| Triethanolamine salt of Miranol C2M anhydrous acid (triethanolamine 1-carboxymethyl-1-carboxyethoxyethyl-2-coco-imidazolinium betaine) | 28.0    |
| Water                                                                                                                                  | 44.0    |

The components of the above formula are blended together and are heated with stirring, to a temperature in the range of 60° to 80° C. to dissolve the gelatin and the various other materials. After about 5 to 10 minutes a clear solution or gel is obtained, which is poured into shaped molds and chilled to 15° C. Upon solidification, which takes about eight minutes, the elastic detergent bar or cake is removed from the mold and is ready for use. The product is satisfactorily elastic and cleans well when it is employed as a bath or hand "soap". It foams very well on initial use and although the foam is diminished upon subsequent uses the bar is a useful washing product and maintains its elasticity throughout repeated washings and dryings. Such bar, containing amphoteric and anionic synthetic organic detergents, with gelatin, does not slough objectionably during use and is less tacky and better foaming than previous bars based on only anionic or amphoteric detergents, respectively.

In a modification of the manufacturing process the hot mixture of bar components is allowed to stand at an elevated temperature in the range of 45° to 55° C. for a period of one hour so as to allow all air bubbles therein to be dissolved or to rise to the top of the mix and separate therefrom before setting of the gel. The products resulting are brighter and clearer in appearance following such deaeration, during which relatively little water and other solvents are evaporated. However, when the temperature of the mixture is raised, e.g., to 60° or 65° to 80° to 90° C., as it is in other embodiments of this example, appreciable loss of water and other volatile materials results and the moisture content of the resulting bar is appreciably diminished. Thus, utilizing a 15 to 30 minute heating period at 80° C., especially in the presence of vacuum, e.g., 250 mm. Hg absolute pressure, 20 to 40%, e.g., 25% of the mix weight is removed. After the evaporation off of 25% of the mix the elastic detergent bar produced includes 11% of triethanolammonium lauryl sulfate, 13% of gelatin, 13% of propylene glycol, 38% of Miranol C2M as the triethanolammonium salt and 25% of water. The elastic detergent bars resulting (deaeration may be effected, too) are firmer, tougher and less liable to shrink upon prolonged exposure to the atmosphere during storage.

When the formula is modified to replace the triethanolammonium lauryl sulfate with the same weight of other suitable anionic detergent, such as ammonium cocomonoglyceride sulfate or a mixture of equal parts of ammonium cocomonoglyceride sulfate and sodium cocomonoglyceride sulfate and when the propylene glycol is replaced by glycerol a product of comparable properties results. Similarly, when the Miranol C2M

salt is replaced by Deriphat 151 or Deriphat 160 or other suitable amphoteric detergent, especially one of the imidazolinium betaine, betaminopropionate or betaiminodipropionate type and when the gelatin is replaced by 15% of 225 g. Bloom type A gelatin (type B may also be used but is not usually as good) essentially the same type of elastic detergent bar results. Similarly, when 2% of potash alum (cross-linking agent) or 1% of urea (denaturant) is present in replacement of a corresponding percentage of water a firmer bar results. When adjuvants are employed, such as fluorescent brighteners; bactericides; emollients; solvents; foaming agents, e.g., lauric myristic diethanolamide; pH adjusting agents, e.g., hydrochloric acid, triethanolamine; perfumes; colorants, including dyes and pigments; and preservatives, they contribute their specific properties to the final bar.

In further modifications of the formula small proportions of dyes and pigments are incorporated to color and opacify the products and gels are molded in chilled molds into the shapes of specific storybook, nursery rhyme, cartoon and animal characters, with the proportions of dyes and pigments employed being about 0.02% for the dyes and about 0.2% for the pigments. The dyed products are transparent or translucent and the pigmented products are opaque. The opacities of the pigmented products are further increased by additions of 1, 2 and 5% of powdered clay to the initial mixture, which also converts the colors to pastels.

The formulas described in this example are modified proportionately ±10%, ±20, and ±30%, within the ranges given and the products resulting are useful elastic detergent products of this invention.

#### EXAMPLE 2

|                                                            | Percent |
|------------------------------------------------------------|---------|
| Ammonium cocomonoglyceride sulfate (47% active ingredient) | 24.2    |
| Triethanolamine salt of Miranol C2M                        | 28.0    |
| Gelatin (300 g. Bloom, type A)                             | 10.0    |
| Propylene glycol                                           | 10.0    |
| Water                                                      | 27.8    |

Elastic detergent bars of the above formula and of such a formula less 25% of water removed in a drying operation after dissolving of the gelatin are made according to the method of Example 1. The bars produced are useful elastic detergent bars for bath use or handwashing and are less tacky and better foaming than similar bars not containing the mixture of anionic and amphoteric detergents. Also, the bars made by a process including removal of moisture, as described, are less liable to shrink on storage exposed to the air than are similar bars containing the greater percentages of moisture. The improved bars, made by reducing the moisture content, analyze about 30% of ammonium cocomonoglyceride sulfate, 35% of triethanolammonium 1-carboxymethyl-1-carboxyethoxyethyl-2-coco-imidazolinium betaine, 13% of gelatin, 12% of propylene glycol and 10% of water. The removal of moisture in the above-described process and other such processes of this invention takes place at a temperature of 30° to 90° C., preferably 40° to 80° C., with the lower temperatures being used most when vacuum is also employed.

## EXAMPLE 3

|                                                                                 | Percent |
|---------------------------------------------------------------------------------|---------|
| Miranol C2M, anhydrous acid                                                     | 21      |
| Triethanolamine                                                                 | 7.5     |
| Propylene glycol                                                                | 10.0    |
| Gelatin (300 g. Bloom, Type A)                                                  | 10.0    |
| Triethanolamine lauryl sulfate<br>(40% active ingredient, aqueous solution)     | 28.5    |
| Ammonium cocomonoglyceride sulfate<br>(47% active ingredient, aqueous solution) | 23.0    |

Following the procedure of Example 1, products of the above formula are made, without moisture removal. They are good elastic detergent bars for both bath use and handwashing and are less tacky and better foaming than similar bars containing either anionic detergent or amphoteric detergent alone. Also, because of their comparatively low moisture content the bars are less liable to shrinkage on storage and when exposed to air than are similar bars containing more moisture.

In normal handwashing use a 100 gram molded bar and molded items in the shapes of cartoon characters, automobiles and animals last for at least 200 handwashings at a water temperature of 40° C., give a copious foam and wash well. They clean well and leave the hands feeling soft, apparently due to the gelatin and amphoteric detergent contents of the products. When 150 gram bars or articles are utilized they last for as many as 20 normal baths, with good foaming throughout such use. During wearing down of the "bars" they substantially retain their general original shapes, colors and foaming and washing abilities.

## EXAMPLE 4

The product of Example 3 is made from an initial mixture which includes 45% of water instead of the 30% in the final product and in the mix of Example 3. The excess moisture is removed during manufacturing by heating for about 45 minutes at a temperature of about 75° C., without vacuum. Comparison of the products of Examples 3 and 4 shows little difference between them except that the product of Example 4 may have the components thereof more uniformly distributed throughout it due to the initial dissolvings of more of them in the aqueous medium before removal of excess moisture. Also, initial mixing and dissolving of the mix of this example is much easier. In a further modification of this example the density of the product is diminished 10%, so that it will float in warm bath water, by distributing small bubbles of air throughout it after removal of the excess moisture from the mixed solution and after cooling of such mix, following the procedure in an application by John C. Carson, Jr. and James A. Bowers, entitled *Elastic Detergent Bar of Improved Elevated Temperature Stability*, filed simultaneously with this application. The product resulting is an excellent "floating soap" for use in the bath tub but unlike soap, it and the other products of this invention leave no bathtub ring and it is a superior floating toy for the child when he takes a bath.

The invention has been described with respect to various embodiments and illustrations thereof but is not to be limited to these because it is evident that one of skill in the art with the present specification before him will be able to utilize substitutes and equivalents without departing from the spirit of the invention.

What is claimed is:

1. An elastic detergent product comprising about 10 to 80% of a mixture of an anionic synthetic organic detergent selected from the group consisting of alkali metal monoglyceride sulfate, ammonium monoglyceride sulfate, triethanolammonium higher fatty alcohol sulfate and mixtures thereof, and an amphoteric synthetic organic detergent, in a proportion between about 1:5 and 5:1, about 5 to 30% of gelatin and about 5 to 60% of water.

15 2. An elastic detergent product according to claim 1 wherein the amphoteric synthetic organic detergent is selected from the group consisting of imidazolinium betaines and betaino dipropionates and mixtures thereof, the proportion of anionic to amphoteric synthetic organic detergent is in the range of 1:4 to 2:1, and the gelatin is a Type A gelatin of 100 to 300 Bloom.

20 3. An elastic detergent product according to claim 2 wherein the mixture of anionic and amphoteric synthetic organic detergents is from 35 to 70% of the bar, the gelatin is of 200 to 300 g. Bloom and is 7 to 25% of the bar and the moisture content is from 10 to 40%.

25 4. An elastic detergent product according to claim 3 which comprises about 3 to 20% of lower dihydric or polyhydric alcohol.

30 5. An elastic detergent product according to claim 3 wherein the anionic synthetic organic detergent is triethanolammonium lauryl sulfate and the amphoteric synthetic organic detergent is triethanolammonium 1-carboxymethyl-1-carboxyethoxyethyl-2-coco-imidazolinium betaine.

6 6. An elastic detergent product according to claim 3 wherein the anionic synthetic organic detergent is ammonium cocomonoglyceride sulfate and the amphoteric synthetic organic detergent is triethanolammonium 1-carboxymethyl-1-carboxyethoxyethyl-2-coco-imidazolinium betaine.

7 7. An elastic detergent product according to claim 4 wherein the anionic synthetic organic detergent is triethanolammonium lauryl sulfate and the amphoteric synthetic organic detergent is triethanolammonium 1-carboxymethyl-1-carboxyethoxyethyl-2-coco-imidazolinium betaine.

45 8. An elastic detergent product according to claim 4 wherein the anionic synthetic organic detergent is ammonium cocomonoglyceride sulfate and the amphoteric synthetic organic detergent is triethanolammonium 1-carboxymethyl-1-carboxyethoxyethyl-2-coco-imidazolinium betaine.

9 9. An elastic detergent product according to claim 7 comprising about 11% of triethanolammonium lauryl sulfate, about 38% of triethanolammonium 1-carboxymethyl-1-carboxyethoxyethyl-2-coco-imidazolinium betaine, about 13% of 300 g. Bloom gelatin, about 13% of propylene glycol, and about 25% of water.

10 10. An elastic detergent product according to claim 8 comprising about 30% of ammonium cocomonoglyceride sulfate, about 35% of triethanolammonium 1-carboxymethyl-1-carboxyethoxyethyl-2-coco-imidazolinium betaine, about 13% of 300 g. Bloom gelatin, about 12% of propylene glycol and about 10% of water.

11 11. An elastic detergent product according to claim 9 which is in the form of a squeezable cartoon character or animal, and which is translucent and squeezable.

12 12. A method of making an elastic detergent product comprising about 10 to 80% of a mixture of anionic and amphoteric synthetic organic detergents in a proportion

between about 1:5 and 5:1, about 5 to 30% of gelatin and about 5 to 40% of water which comprises heating together a mixture of such components, with additional water to promote solubilization of the gelatin and evaporating off water in a proportion from 15 to 50% of the weight of the mixture.

13. A method according to claim 12 wherein the elastic detergent product comprises about 35 to 65% of a mixture of triethanolammonium lauryl sulfate and triethanolammonium 1-carboxymethyl-1-carboxyethoxyethyl-2-coco-imidazolinium betaine in a proportion within the range of 1:4 to 2:1, 7 to 25% of a type A gelatin of 100 to 300 g. Bloom and 10 to 40% of water which comprises heating a mixture of such components in an aqueous medium containing 25 to 60% of water until the gelatin is dissolved, continuing heating until 20 to 40% of the mix weight of water is removed, deaerating the composition and pouring it into a mold.

14. A method according to claim 12 wherein the elastic detergent product comprises about 35 to 70% of 20

5 a mixture of ammonium cocomonoglyceride sulfate and triethanolammonium 1-carboxymethyl-1-carboxyethoxyethyl-2-coco-imidazolinium betaine in a proportion within the range of 1:4 to 2:1, 7 to 25% of a type A gelatin of 100 to 300 g. Bloom and 10 to 40% of water which comprises heating a mixture of such components in an aqueous medium containing 25 to 60% of water until the gelatin is dissolved, continuing heating until 20 to 40% of the mix weight of water is removed, deaerating 10 the composition, pouring it into a mold, chilling and solidifying it and removing it from the mold.

15. A process according to claim 14 wherein the product comprises about 30% of ammonium cocomonoglyceride sulfate and about 38% of triethanolammonium-1-carboxyethyl-1-carboxyethoxyethyl-2-coco-imidazolinium betaine, and is in the form of a squeezable cartoon character or animal which is translucent and squeezable, and the chilling is to solidification.

\* \* \* \* \*

25

30

35

40

45

50

55

60

65